

May 22, 1956

G. L. DENISTON

2,746,880

ADHESIVE COTTON ARTICLE AND METHOD OF MAKING SAME

Original Filed Aug. 14, 1951



INVENTOR  
GEORGE L. DENISTON  
BY *G. L. Deniston*  
ATTORNEYS

# United States Patent Office

2,746,880

Patented May 22, 1956

1

2,746,880

## ADHESIVE COTTON ARTICLE AND METHOD OF MAKING SAME

George L. Deniston, Dayton, Ohio, assignor to The Commonwealth Engineering Company of Ohio, Dayton, Ohio, a corporation of Ohio

Original application August 14, 1951, Serial No. 241,740, now Patent No. 2,706,690, dated April 19, 1955. Divided and this application September 22, 1952, Serial No. 319,904

12 Claims. (Cl. 117—63)

This invention relates to a process of treating cotton threads, yarns and fabrics with dextran and its derivatives and to the products produced thereby.

This application is a division of application Serial No. 241,740, filed August 14, 1951, now U. S. Patent Serial No. 2,706,690, and assigned to the same assignee as the present invention.

Dextran is a water soluble colloidal material produced by the action of microorganisms on sucrose bearing materials and may be converted into dextran ethers and esters as described in U. S. Patents 2,344,179, 2,203,702 and 2,385,553.

This invention contemplates the provision of a novel process for the impregnation and coating of cotton materials with dextran and its derivatives.

The invention contemplates the provision of a new product wherein cotton provides a strength core and material impregnated therein and coated thereon provides an outer shell resistant to ordinary chemical attack but which may be rendered sufficiently tacky by selected solvents for the securing of good adhesions in many materials of commerce.

More particularly, in the process of invention cotton in the form of a thread, yarn or fabric is treated with dextran, dissolved in a solvent, to secure penetration of the dextran into the fibers, and thereafter the dextran bearing cotton is treated with an alkylating agent in an alkaline solution and then subjected to a heating step to form a product resistant to chemical action but selectively attacked by particular solvents. An additional feature of the process, particularly as related to commercial yarn and fabrics as used in rubber and plastic industries, is the substantial elimination of residual stretch therefrom by the heating of the composite body under tensile conditions.

While I prefer to use a combination of sodium hydroxide and water as the dextran solvent, due to the efficiency of this combination in the effecting of a swelling of the cotton fibers to thereby permit maximum penetration of the dextran, other solvents, e. g. water alone, water and sodium carbonate, a dilute acetic acid solution or dilute solutions of the mineral acids such as HCl and H<sub>2</sub>SO<sub>4</sub> may suitably be employed.

The alkylating agent for the dextran, which is utilized to substitute or add an alkyl group into the dextran, may include: the organic halides such as methyl, ethyl, propyl; isopropyl or benzyl halides; the alkyl sulphates such as diethyl sulphate; tri-ethyl phosphate; and aryl sulfonic alkyl esters such as the ethyl ester of p-toluene sulfonic acid.

The alkylating agent is employed in alkaline solution and this alkali is preferably sodium or potassium hydroxide, sodium carbonate or an organic alkali.

The product of the process of invention may comprise, for example, a destretched yarn having the cotton core surrounded by the benzyl ether of dextran which is insoluble in and substantially unaffected by H<sub>2</sub>O, alkalis, mineral acids, and the lower aliphatic alcohols, but which when treated with acetone, dioxane, benzene or toluene

2

becomes tacky. Thus this destretched yarn has a particular utility in power transmission belt structures where it may be laminated with rubber and cured thereto. Similarly a fabric treated by the process of invention attains qualities suitable for lamination with resinous materials.

The invention will be more fully understood by reference to the following specific examples and the drawing wherein:

Figure 1 illustrates the apparatus used in the process of invention;

Figure 2 is a view of the grooved roller in Figure 1;

Figure 3 is a partial plan view of the apparatus of Figure 1; and

Figure 4 is a plan view of the grooved tapered roller shown in the oven of Figure 1.

### Example I

There is shown in Figure 1 a tank or vat 1 containing a dextran solution 2, the solution containing by weight approximately 40% dextran of any molecular weight, 55% water and about 5% of sodium hydroxide. A cotton yarn 3 is shown passing continuously from bobbin 4, mounted on roll 5, into the solution 2 where it is guided between rolls 6 and 7, which are adapted to be driven independently by means not shown at speeds differing by about 30%, the roll 7 having the greater velocity. The rolls 6 and 7 are multi-grooved as shown in Figure 2 in order that the time of passage of the yarn through the solution may be readily controlled, by utilization of a selected number of grooves for particular size yarns.

The yarn is shown in Figure 1 as passing from solution 2 over roll 8 into bath 9 containing alkaline aralkyl halide solution 10 having by weight approximately 30% of benzyl chloride, 9% of sodium hydroxide and 61% water. The wetted and impregnated yarn 3 passes over rolls 20 and 21 which are grooved similarly to rolls 6 and 7 and after a multi pass through the solution, as more clearly shown in Figure 3, enters a heated oven 12 over roller 11. A hollow conical die 13 is positioned between bath 9 and oven 12 to remove any excess material present on the yarn before it passes to the heating operation.

The oven 12 is provided with grooved rollers 14, 15, roller 15 being driven at a speed about 30% in excess of that of roller 14, and the roller 15 having grooves of progressively (Figure 4) increasing diameter, from end 16 to end 17, to facilitate the destretching of the yarn. After curing the yarn is wound up on coil 18 mounted on stand 19.

When impregnating and coating the yarn is passed through bath 2 under tension if desired although the same is not necessary but does assist in the ultimate de-stretching of the yarn and the dextran pick up is somewhat greater if tension is employed. In solution 10 the dextran and aralkyl halide initiate a reaction which is completed in oven 12 at temperatures of about 130 to 140° C.

The finished product has substantially no stretch retained therein and due to the coating resists moisture thus preventing shrinkage effects from occurring in the yarn rendering the product particularly useful where constant yarn length under varying humidity conditions is essential. Since the product is also resistant to alcohols, the mineral acids, and alkalis, it may be employed under conditions where such resistance is beneficial.

It will be clear from the foregoing that the degree of impregnation of the yarn may be controlled by controlling the solution concentrations particularly the dextran. Furthermore a coating may be applied over the yarn to completely sheath the same by utilizing viscous solution.

### Example II

The apparatus described in connection with Example I may be readily modified to permit the coating of a cotton

fabric with an ethyl dextran which is resistant to water, the mineral acids, and alkalis, but soluble in the alcohols.

The dextran may in this instance be solved in a weak sodium hydroxide, and an efficient mixture would contain:

50% dextran  
40% water  
10% sodium hydroxide

The fixing solution may contain:

50% di-ethyl sulphate  
30% water  
20% sodium hydroxide

The procedure is essentially the same as set forth in Example I, the heating temperature however being of the order of 100-115° C.

It will be understood that while there have been given herein certain specific examples of the practice of this invention, it is not intended thereby to have this invention limited to or circumscribed by the specific details of materials, proportions or conditions herein specified, in view of the fact that this invention may be modified according to individual preference or conditions without necessarily departing from the spirit of this disclosure and the scope of the appended claims.

I claim:

1. An adhesive yarn consisting of a cotton core impregnated and coated with a substance selected from the group consisting of alkyl and aralkyl ethers of dextran, said core being set in substantially non-stretchable condition by the dextran ether, and said ether being in adhesive condition in and on the core as a result of solvent treatment thereof in situ in the yarn.

2. An adhesive yarn consisting of a cotton core impregnated and coated with an ethyl ether of dextran, said core being set in substantially non-stretchable condition by the dextran ether, and said ether being in adhesive condition in and on the core as a result of solvent treatment thereof in situ in the yarn.

3. An adhesive yarn consisting of a cotton core impregnated and coated with a benzyl ether of dextran, said core being set in substantially non-stretchable condition by the dextran ether, and said ether being in adhesive condition in and on the core as a result of solvent treatment thereof in situ in the yarn.

4. A fabric comprising adhesive yarns consisting of a cotton core coated and impregnated with a substance selected from the group consisting of alkyl and aralkyl ethers of dextran, said core being set in substantially non-stretchable condition by the dextran ether, and said ether being in adhesive condition in and on the core as the result of solvent treatment thereof in situ in the fabric.

5. A power transmission belt comprising yarns consisting of a cotton core coated and impregnated with a substance selected from the group consisting of alkyl and aralkyl ethers of dextran, said core being set in substantially non-stretchable condition by the dextran ether, and said ether being in adhesive condition in and on the core as the result of solvent treatment thereof in situ in the belt.

6. A power transmission belt comprising yarns consisting of a cotton core coated and impregnated with a benzyl ether of dextran, said core being set in substantially non-stretchable condition by the dextran ether, and said

ether being in adhesive condition in and on the core as the result of solvent treatment thereof in situ in the belt.

7. The method of producing an adhesive cotton yarn which comprises treating a cotton yarn with an aqueous alkaline solution of dextran, then treating the dextran-impregnated cotton yarn with an aqueous alkaline solution of an etherifying agent selected from the group consisting of alkylating and aralkylating agents, heating the impregnated yarn to complete reaction between the etherifying agent and the dextran in situ in the yarn, and thereafter treating the yarn with a solvent for the dextran ether to activate the ether to adhesive condition.

8. The method of producing an adhesive cotton yarn which comprises treating a cotton yarn with an aqueous alkaline solution of dextran, then treating the dextran-impregnated cotton yarn with an aqueous alkaline solution of a benzyl ether of dextran, heating the impregnated yarn to a temperature of 130° C. to 140° C. to complete reaction between the etherifying agent and the dextran in situ in the yarn, and thereafter treating the yarn with acetone to activate the ether to adhesive condition.

9. The method of producing an adhesive cotton yarn which comprises treating a cotton yarn with an aqueous alkaline solution of dextran, then treating the dextran-impregnated cotton yarn with an aqueous alkaline solution of a benzyl ether of dextran, heating the impregnated yarn to a temperature of 130° C. to 140° C. to complete reaction between the etherifying agent and the dextran in situ in the yarn, and thereafter treating the yarn with dioxane to activate the ether to adhesive condition.

10. The method of producing an adhesive cotton yarn which comprises treating a cotton yarn with an aqueous alkaline solution of dextran, then treating the dextran-impregnated cotton yarn with an aqueous alkaline solution of a benzyl ether of dextran, heating the impregnated yarn to a temperature of 130° C. to 140° C. to complete reaction between the etherifying agent and the dextran in situ in the yarn, and thereafter treating the yarn with benzene to activate the ether to adhesive condition.

11. The method of producing an adhesive cotton yarn which comprises treating a cotton yarn with an aqueous alkaline solution of dextran, then treating the dextran-impregnated cotton yarn with an aqueous alkaline solution of a benzyl ether of dextran, heating the impregnated yarn to a temperature of 130° C. to 140° C. to complete reaction between the etherifying agent and the dextran in situ in the yarn, and thereafter treating the yarn with toluene to activate the ether to adhesive condition.

12. The method of claim 7 in which the treatment with the aqueous solution of the etherifying agent is performed while the yarn is under tension.

#### References Cited in the file of this patent

#### UNITED STATES PATENTS

|           |               |       |               |
|-----------|---------------|-------|---------------|
| 148,319   | Newton        | ----- | Mar. 10, 1874 |
| 2,126,936 | Wall          | ----- | Aug. 16, 1938 |
| 2,203,705 | Stahly et al. | ----- | June 11, 1940 |
| 2,236,386 | Stahly et al. | ----- | Mar. 25, 1941 |
| 2,344,179 | Stahly        | ----- | Mar. 14, 1944 |
| 2,486,399 | Gagarine      | ----- | Nov. 1, 1949  |
| 2,503,624 | Luaces        | ----- | Apr. 11, 1950 |